

# United States Patent Office

2,971,912

Patented Feb. 14, 1961

1

2,971,912

## LUBRICATING OIL COMPOSITIONS

John Scotchford Elliott, and Eric Descamp Edwards, London, England, assignors to Castrol Limited, a British company

No Drawing. Filed May 13, 1957, Ser. No. 658,519

Claims priority, application Great Britain May 14, 1956

11 Claims. (Cl. 252—46.7)

The present invention comprises improvements in or relating to lubricating compositions and relates particularly to fluid lubricants suitable for use over a wide range of temperatures and under a variety of conditions.

It is an object of the present invention to provide lubricating compositions suitable for use in internal combustion engines or other mechanisms where high temperatures are involved e.g. in the lubrication of gas turbines, especially the propeller turbine type where the lubricant is required to lubricate not only the bearings but also the reduction gearing, said lubricating compositions also being stable and fluid at low or very low temperatures e.g. down to  $-40^{\circ}$  F. or even  $-80^{\circ}$  F.

It has already been proposed to employ as lubricants (especially suited for use at low temperatures) certain diesters of aliphatic dicarboxylic acids with branched-chain aliphatic alcohols, a number of such esters being described in the Journal entitled "Industrial and Engineering Chemistry," April 1947, p. 484 to p. 497.

Recent improvements in the design of gas turbine engines have increased the severity of the demands made upon the lubricant, which must have good oxidation resistance at high temperatures, e.g. of the order of  $200^{\circ}$  C., at the same time being non-corrosive towards metals used in the construction of the turbine engines, e.g. steel, copper, brass, magnesium, aluminium and cadmium plated steel. It must also possess a high load-carrying capacity, in order to provide adequate lubrication of the reduction gearing in the propeller-turbine type of engines.

In our United States patent application No. 456,063, now U.S. Patent No. 2,836,565, we have disclosed the fact that di(hydroxyaryl) thioethers are a class of thermally stable compounds which may be added to the esters above referred to in order to improve their oxidation resistance at high temperatures.

Other examples of effective antioxidants are phenothiazine and some of its derivatives as described in the Journal entitled "Industrial and Engineering Chemistry," December 1950, p. 2479 to p. 2489.

Another class of antioxidants which are quite effective at high temperatures are the dialkyl selenides of relatively high molecular weight.

While these additives are all effective to a greater or less degree in inhibiting the oxidation of ester-type synthetic lubricants, they suffer from the disadvantage of tending to break down at high temperatures with the consequent formation of products which are corrosive to cuprous metals and silver. Thus, for example, ester-type synthetic lubricants containing phenothiazine may, under certain conditions, produce at elevated temperatures an undesirable amount of tarnishing of copper and cuprous metals or silver, whilst di(hydroxyaryl) thioethers react with copper and cuprous metals to form copper derivatives which at very high temperatures, e.g. of the order of  $280^{\circ}$  C., tend to decompose with the formation of copper sulphides. As pointed out in United States patent application No. 456,063 the corrosive tendencies of di(hydroxyaryl) thioethers towards cuprous metals may be

2

reduced by the inclusion in the blend of certain basic aliphatic, alicyclic or heterocyclic amines, but these compounds are not completely effective at the very high temperatures above referred to.

5 We have now found that by the inclusion in ester-type synthetic lubricants containing one or more antioxidants of the foregoing classes of a minor proportion of one or more heterocyclic compounds as hereinafter defined, effective protection of cuprous metals and silver can be achieved even at high temperatures.

Accordingly, the present invention provides a lubricating composition comprising a neutral ester or mixture of esters as hereinafter defined and a minor proportion of (a) a compound having antioxidant properties at elevated

15 temperatures and containing the group  $—C—S—C—$  or  $—C—Se—C—$  and (b) an organic heterocyclic compound containing two or three nitrogen atoms and one  $—C=C—$  linkage in a five-membered heterocyclic ring.

The term "neutral ester" used throughout the specification is to be understood as referring to esters having an acidity not exceeding 1 mg. KOH per gm.

The esters which are suitable for use as the lubricant base in accordance with the present invention are substantially neutral saturated organic carboxylic acid esters having a viscosity index of at least 100, a pour point or freezing point not exceeding  $-40^{\circ}$  F., a boiling or decomposition temperature not less than  $600^{\circ}$  F. and a flash point not less than  $350^{\circ}$  F. It will be understood that mixtures of esters may be employed comprising individual esters which have freezing points above  $-40^{\circ}$  F. and viscosity indices below 100, provided that the mixture itself has the desired properties.

The preferred esters have the general formula



wherein R is a saturated aliphatic or cycloaliphatic hydrocarbon radical having from 2 to 8 carbon atoms, and 40 R<sub>1</sub> and R<sub>2</sub> are the same or different and are branched-chain alkyl or alkyl-substituted cycloalkyl radicals having at least 4 carbon atoms. Examples of the radical R are (CH<sub>2</sub>)<sub>n</sub> (where n is an integer from 2 to 8) and



50 While esters having the above general formula are preferred, it is also within the scope of the invention to employ esters obtained by esterifying the dicarboxylic acids with a mixture of an alcohol and a glycol to give complex esters having the general formula



wherein R, R<sub>1</sub> and R<sub>2</sub> are as defined above and



is a glycol or polyglycol having not more than about 12 carbon atoms.

65 Other types of complex esters which may be employed are prepared by esterifying a dicarboxylic acid (1 mol) with a glycol (2 mols) and a monocarboxylic acid (2 mols) or with 1 mol each of a glycol, a monocarboxylic acid and a monohydric alcohol or with 2 mols each of a hydroxy-acid and an alcohol. Still other types of complex ester may be prepared by esterifying a glycol (1 mol)

with a hydroxy-acid (2 mols) and a monocarboxylic acid (2 mols).

Other esters which may be suitable in certain circumstances are prepared by esterifying a glycol or polyglycol (1 mol) with 2 mols of a monocarboxylic acid, while still other esters may be obtained by completely esterifying with a suitable monocarboxylic acid polyhydric alcohol such as trimethylol propane or pentaerythritol.

It is to be understood that in the foregoing formulae the radicals  $R_1$ ,  $R_2$  and  $R_3$  may, if desired, contain ether oxygen linkages. The mono-, di- and polyhydric alcohols, and the monocarboxylic acids employed in the preparation of the complex esters may also contain ether oxygen linkages. The esters should, however, be free from elements other than carbon hydrogen and oxygen.

The preferred diesters are derived from succinic, pyrotartaric, glutaric, adipic, pimelic, suberic, azelaic, sebacic and pinic acids, specific esters being:

Di(1-methyl-4-ethyl octyl) glutarate  
 Di(2-ethyl hexyl) adipate  
 Di(3-methyl butyl) azelate  
 Di(2-ethyl hexyl) azelate  
 Di(2-ethyl hexyl) sebacate  
 Di(3:5:5-trimethylhexyl) sebacate  
 Di(3:5:5-trimethylhexyl) azelate  
 2 ethyl hexyl 1-methyl heptyl sebacate  
 Di(2-ethyl hexyl) pinate  
 Di( $C_{10}$  Oxo) adipate  
 Bis(diethylene glycol monobutyl ether) adipate  
 Di(1-methyl-4-ethyl octyl) sebacate  
 2-ethyl hexyl 3:5:5 trimethyl hexyl sebacate.

Whereas the majority of esters falling within the foregoing class possess both a high viscosity index and low pour-point, certain of them e.g. di(1:3 dimethyl butyl) adipate, di(3-methyl butyl) sebacate have relatively high freezing points (above 0° F.), and therefore would not normally be suitable for the purpose of this invention, except in admixture with other esters of lower freezing point.

It will be understood that different esters may be selected according to the conditions under which the lubricant is to be used. Thus for use at very high temperatures it will be preferred to employ the esters of high molecular weight and particularly the higher branched-chain di-esters of azelaic and sebacic acid.

The complex esters which may be employed are preferably prepared by esterifying 2 mols of the dicarboxylic acid, 2 mols of the branched-chain aliphatic or alkyl-substituted cycloaliphatic alcohol, and not more than 1 mol of glycol. Examples of glycols which may be used are ethylene, propylene and hexylene glycols. 2-ethyl-1:3 hexanediol and the poly glycols, e.g. diethylene, triethylene, and tetraethylene glycol.

When a monocarboxylic acid is used in preparing a complex ester this should be a straight or branched-chain aliphatic acid having from 2 to 10 carbon atoms inclusive.

Specific examples of suitable complex esters which may be employed in accordance with the present invention are:

Ester prepared from ethylene glycol (1 mol), adipic acid (2 mols) and 2-ethyl hexanol (2 mols).

Ester prepared from tetraethylene glycol (1 mol), sebacic acid (2 mols), and 2-ethyl hexanol (2 mols).

Ester prepared from 2-ethyl-1:3 hexanediol (1 mol), sebacic acid (2 mols), and 2-ethyl hexanol (2 mols).

Ester prepared from diethylene glycol (1 mol), adipic acid (2 mols) and n-butanol (2 mols).

Ester prepared from polyglycol 200 (1 mol), sebacic acid (2 mols) and ethylene glycol mono (2-ethyl butyl) ether (2 mols).

Ester prepared from sebacic acid (1 mol), tetraethylene glycol (2 mols) and caproic acid (2 mols).

Ester prepared from triethylene glycol (1 mol) adipic

acid (1 mol), n-caproic acid (1 mol) and 2-ethyl hexanol (1 mol).

Ester prepared from sebacic acid (1 mol), lactic acid (2 mols) and n-butanol (2 mols).

Ester prepared from tetraethylene glycol (1 mol), lactic acid (2 mols) and butyric acid (2 mols).

Examples of suitable glycol and polyhydric alcohol esters of monocarboxylic acids which may be employed are:

10 Triethylene glycol di(2-ethyl hexanoate)

Hexanediol 1,6 di(2-ethyl hexanoate)

Trimethylol propane tri-n-octanoate.

The antioxidants, additive (a), consist as already indicated of organic compounds having antioxidant properties at elevated temperatures and containing the group

15  $-\text{C}-\text{S}-\text{C}-$  or  $-\text{C}-\text{Se}-\text{C}-$ . Whilst a wide variety of compounds of this general type, e.g. the aliphatic sulphides, have certain antioxidant properties at elevated temperatures, many compounds have serious limitations 20 at really high temperatures, e.g. of the order of 175° C., such as are encountered in the lubrication of gas turbine engines.

The preferred antioxidants, which are effective to a greater or less degree at high temperatures are of three

25 different types:

(i) Di(hydroxyaryl) thioethers of the type described and exemplified in our United States patent application No. 456,063 and particularly di(hydroxyphenyl) thioethers in which the benzene nuclei are unsubstituted or 30 substituted only by short-chain alkyl radicals.

(ii) Dibenzothiazines having good antioxidant properties at elevated temperatures.

The dibenzothiazines are preferably dibenzo 1,4 thi- 35 azines. The benzo radicals may contain further substitu-

ents e.g. alkyl or aryl groups, or halogens.

The selenium analogues of these compounds may also be employed i.e. dibenzoselenazines.

Typical examples of compounds falling within this class are:

Phenothiazine (2,3,5,6 dibenzothiazine)

Phenoselenazine

Phenothiazone-3

Phenothiazine-5-oxide

10-10' diphenothiazine

10-benzyl phenothiazine

7-benzo (c) phenothiazine

3,7 difluorophenothiazine

(iii) Dialkyl selenides having at least 20 carbon atoms e.g. dilauryl selenide and dicetyl selenide.

45 50 The antioxidants employed in the present invention should have a decomposition temperature of at least 200° C. and have adequate solubility in the esters in which they are to be dissolved.

The organic heterocyclic compounds, additive (b), 55 are imidazoles, pyrazoles or 1,2,3 triazoles. They contain respectively the groups



where R=H, or an alkyl, alkenyl or aryl group.

The compounds selected should not boil or decompose below 200° C., and preferably not below 300° C., and they should be soluble in the lubricant in the proportions in which they are intended to be employed.

Specific examples of such additives are:

Imidazole  
Benzimidazole  
Pyrazole  
Benzotriazole  
2-methyl benzimidazole  
3:5 dimethyl pyrazole  
Indazole

The major proportion of the lubricating composition of the present invention consists of the esters hereinbefore described. The antioxidants may be employed in proportions ranging from 0.05 percent to 5.0 percent, and preferably from 0.1 percent to 2.0 percent, by weight on the weight of the final composition. Generally the organic heterocyclic compounds will be employed in relatively small amounts e.g. from 0.01 percent to 2.0 percent, and preferably from 0.05 percent to 0.5 percent, by weight on the weight of the final composition.

It is also within the scope of the invention to include lubricants in which a certain amount of mineral oil is added to the composition. The amount added and type of mineral oil will depend largely upon the pour-point required for the particular application in mind, but in any case the amount of mineral oil present should not exceed 20% by weight on the weight of the final composition.

In one form of the present invention the dicarboxylic acid diesters of the type described are thickened by the addition of polymers of esters of acrylic or alkyl-substituted acrylic acids, e.g. polymerised n-butyl or higher esters of methacrylic acid. Compositions of this type can be produced having sufficiently high viscosities combined with very low pour-points.

The polymers are employed in proportions of from 1% to 15% preferably from 5% to 10%, by weight on the weight of the final composition.

Examples of polymers which may be employed are the polymerised n-hexyl, 3:5:5 trimethyl hexyl and lauryl esters of methacrylic acid, and various commercially available materials sold under the trade name "Acryloid." It is preferred to use polymers which are not only freely soluble in the diester lubricants but also miscible with mineral oil.

Alternatively polyesters, e.g. polypropylene glycol sebacates of varying molecular weights may be used in place of the polymers of esters of acrylic or alkyl-substituted acrylic acids in order to increase the viscosity of the lubricating composition.

In a further form of the present invention there may be included in the lubricating composition certain amines in order to reduce the corrosion of cuprous metals and to impart to the blend increased stability towards oxidation. Examples of suitable amines are described in our United States patent application No. 456,063.

Generally these amines will be employed in relatively small amounts, e.g. from 0.01 to 1.0 percent, and preferably from 0.05 to 0.5 percent, by weight on the weight of the final composition.

- 5 In order to enhance the load-carrying capacity of the lubricating compositions of the present invention particularly when such compositions are to be used for gas turbine lubrication there may be added to the compositions a proportion of one or more load-carrying additives. Thus there may be included in the composition a proportion of the neutral organic phosphate or phosphite esters disclosed in our United States patent application No. 483,824, now U.S. Patent No. 2,820,766.

15 Examples of such compounds include

- Tri(n-butyl) phosphate  
Tri(2-ethyl hexyl) phosphate  
Tri-o-tolyl phosphate  
Tri-m-tolyl phosphate  
20 Tri(p-tertiary amyl phenyl) phosphate  
Tri(methyl cyclohexyl) phosphate  
Tri(n-butyl phosphite)  
Tri phenyl phosphite  
Tritolyl phosphite  
25 Tri cyclohexyl phosphite  
Di(3-carbomethoxy-4-hydroxyphenyl) thioether ditolyl phosphite

The phosphate ester may be employed in an amount of 30 from 0.5 percent to 10 percent, preferably from 1.0 percent to 5.0 percent, by weight on the weight of the final composition and the phosphite ester may be employed in an amount of from 0.1 percent to 5.0 percent, preferably from 0.25 percent to 2.0 percent, by weight on the weight of the final composition.

35 Other additives may be included if desired, e.g. rust inhibitors such as very small amounts of metal petroleum sulphonates, or other known compounds capable of inhibiting rust formation in the presence of water.

40 Specific compositions which may be employed in accordance with the present invention are exemplified in the tables of test results which follow.

In one simple test method which was employed, strips of copper foil, approximately 2" x 1/2", polished with carborundum powder, were placed in test-tubes which were partially filled with the oil under test, the copper strip being completely immersed. The test-tube was placed in a beaker of oil and heated in an oven.

45 In a first series of tests carried out according to this procedure, small proportions of different corrosion inhibitors were added to a blend consisting of di(3:5:5 trimethylhexyl) sebacate (D.N.S.) containing 1.0 percent of a technical grade of di(3-methyl-4-hydroxyphenyl) thioether. The results are summarised in Table 1.

Table 1

| Test No. | Inhibitor              | Percent of Inhibitor | Appearance of copper strip after—          |                                             |
|----------|------------------------|----------------------|--------------------------------------------|---------------------------------------------|
|          |                        |                      | 4 hours                                    | 22 hours                                    |
| 1.       | None                   |                      | Dark brown/black, smooth                   | Black, flaky.                               |
| 2.       | Benzotriazole          | 0.1                  | Brown deposit, on light copper background. | Dark brown.                                 |
| 3.       | Imidazole              | 0.1                  | Brown/dark peacock                         | Brown/very dark peacock.                    |
| 4.       | Benzimidazole          | 0.2                  | Very light peacock, light brown deposit.   | Light peacock, medium brown deposit.        |
| 5.       | Pyrazole               | 0.3                  | Light brown; white powdery deposit.        | Dark brown.                                 |
| 6.       | 3:5 Dimethyl pyrazole  | 0.5                  | Light stain                                | Smooth brown.                               |
| 7.       | Indazole               | 0.3                  | Heavy greenish brown powdery deposit.      | Heavy dark brown deposit.                   |
| 8.       | 2-Methyl benzimidazole | 0.2                  | Light peacock                              | Light peacock with some dark brown deposit. |

All inhibitors added to D.N.S.+1.0% di(3-methyl-4-hydroxy-phenyl) thioether.  
Temperature 150° C.  
Duration of test 22 hours

It will be seen from Table I that all the compounds tested were effective to a greater or lesser extent, in inhibiting the attack of copper by technical di(3-methyl-4-hydroxyphenyl) thioether, or by impurities contained therein, at 150° C.

A second series of tests was carried out under the same conditions, but at 200° C. for 6 hours, the results being summarised in Table II. In this series of tests, two blends were tested, with and without the addition of 0.2% of benzotriazole.

Antioxidants of the dibenzothiazine type, such as phenothiazine, possessed greater thermal stability than the di(hydroxyaryl) thioethers and produced no more than light staining of the copper under the foregoing test conditions, even at 250° C. (6 hours).

It was observed, however, that if the test strips were only partially immersed in the oil, considerable attack of the copper took place above the oil, and particularly 10 at the oil-air interface. This attack could be appreciably

Table II

| Test No. | Composition of blend                                                                                                                                                                                                                                                                                                                                                                                   | Inhibitor   | Appearance of copper strip                   |
|----------|--------------------------------------------------------------------------------------------------------------------------------------------------------------------------------------------------------------------------------------------------------------------------------------------------------------------------------------------------------------------------------------------------------|-------------|----------------------------------------------|
| 9.....   | 45% D.O.S.<br>45% D.N.S.<br>6% Polynonyl methacrylate<br>3% Tri-m-tolyl phosphate<br>1% p,p-Dihydroxy-diphenyl thioether<br>45% D.O.S.<br>45% D.N.S.                                                                                                                                                                                                                                                   | Absent....  | Light brown stain.                           |
| 10.....  | 6% Polynonyl methacrylate<br>3% Tri-m-tolyl phosphate<br>1% p,p-Dihydroxy-diphenyl thioether<br>(88% Di(2-ethyl hexyl) adipate<br>10% Poly propylene sebacate<br>2% Di(3-methyl-4-hydroxyphenyl) thioether (technical)<br>+0.1% Dicyclohexylamine<br>(88% Di(2-ethyl hexyl) adipate<br>10% Poly propylene sebacate<br>2% Di(3-methyl-4-hydroxyphenyl) thioether (technical)<br>+0.1% Dicyclohexylamine | Present.... | Matt copper colour, with some white deposit. |
| 11.....  |                                                                                                                                                                                                                                                                                                                                                                                                        | Absent....  | Dark brown, 10% black.                       |
| 12.....  |                                                                                                                                                                                                                                                                                                                                                                                                        | Present.... | Medium brown.                                |

Temperature..... 200° C.

Duration of test..... 6 hours.

Inhibitor..... 0.2% of benzotriazole.

In this table, "DOS" represents di(2-ethyl hexyl) sebacate, the "polynonyl methacrylate" used was poly (3:5:5-trimethyl hexyl) methacrylate, and the poly propylene sebacate was a commercially available material known as "Reoplex 100" ("Reoplex" is a registered trademark).

In Table II, comparison between Tests Nos. 9 and 11 indicates that the principal causes of copper staining by

reduced by the inhibitors of the present invention, as demonstrated in Table III.

Table III

| Test No. | Composition of blend                                                                                                      | Inhibitor                       | Appearance of copper strip                                             |
|----------|---------------------------------------------------------------------------------------------------------------------------|---------------------------------|------------------------------------------------------------------------|
| 13.....  | 56.5% DOS<br>40% Complex Ester<br>3% Polynonyl methacrylate<br>0.5% Phenothiazine (technical)<br>56.5% DOS                | None.....                       | Black flaky deposit at and above interface.                            |
| 14.....  | 40% Complex Ester<br>3% Polynonyl methacrylate<br>0.5% Phenothiazine (technical)<br>56.5% DOS                             | Benzimidazole (0.2%)....        | Smooth peacock above oil with brown line at interface.                 |
| 15.....  | 40% Complex Ester<br>3% Polynonyl methacrylate<br>0.5% Phenothiazine (technical)<br>94% ONS                               | Benzotriazole (0.05%)....       | Smooth brown above oil with black line at interface.                   |
| 16.....  | 5% Mineral Oil A<br>0.25% Calcium petroleum sulphonate (20% in mineral oil)<br>0.75% 7-Benzo (c) phenothiazine<br>94% ONS | None.....                       | Heavy dark brown flaky deposit at interface and just above.            |
| 17.....  | 5% Mineral Oil A<br>0.25% Calcium petroleum sulphonate (20% in mineral oil)<br>0.75% 7-Benzo (c) phenothiazine            | 2-Methyl benzimidazole (0.05%). | Light brown smooth above oil, with dark line at interface. No deposit. |

Temperature..... 250° C.

Duration of test..... 6 hours

Copper strips partially immersed.

di(hydroxyaryl) thioethers at temperatures of the order of 150° to 200° C. are impurities, the relatively pure compound in Test No. 9 giving only a light brown stain, whereas the compound used in Test No. 11 gave some blackening even in the presence of dicyclohexylamine. In both cases, however, a manifest improvement was obtained by the introduction of benzotriazole.

In a similar test at 200° C. with a silver specimen, a solution of 1% of di(3-methyl-4-hydroxyphenyl) thioether in D.O.S. produced a dark tarnish on the silver, which did not form when 0.2% of benzotriazole was added to the blend.

65 In Table III, the complex ester was of the type obtained by esterifying a dicarboxylic acid (2 mols) with a branched-chain aliphatic alcohol (2 mols) and a glycol (1 mol), and was a material known as "Paraplex AP-52" (Paraplex is a registered trademark). "ONS" represented 70 2-ethyl hexyl 3:5:5 trimethyl hexyl sebacate. Mineral oil A was a solvent-refined mineral oil of viscosity about 65 seconds Redwood I at 140° F.

A further series of tests was now carried out employing the oxidation/corrosion test procedure described in 75 Ministry of Supply Material Specification No. D. Eng.

R.D. 2487 (Issue No. 2, dated 1st January, 1954), paragraph 7-4. This test was a combined oxidation and corrosion test designed to measure the tendency of an oil to develop corrosive oxidation products at elevated temperatures. The results are summarised in Table IV.

wherein R is a radical selected from the group consisting of saturated aliphatic and cycloaliphatic hydrocarbon radicals having from 2 to 8 carbon atoms, and R<sub>1</sub> and R<sub>2</sub> are radicals selected from the group consisting of branched-chain alkyl and alkyl-substituted cycloalkyl rad-

Table IV

[All tests were carried out for 22 hours at 140° C.]

| Test No. | Ester or Ester Blend                                                                                                                                                                                                                                                                                                                                                   | Additives                                                                                      | Cadmium plated steel test-piece with copper catalyst |                                   |                                                  | Copper test-piece with steel catalyst |                   |                                                    |
|----------|------------------------------------------------------------------------------------------------------------------------------------------------------------------------------------------------------------------------------------------------------------------------------------------------------------------------------------------------------------------------|------------------------------------------------------------------------------------------------|------------------------------------------------------|-----------------------------------|--------------------------------------------------|---------------------------------------|-------------------|----------------------------------------------------|
|          |                                                                                                                                                                                                                                                                                                                                                                        |                                                                                                | Wt. change (mgs.)                                    | Colour of—                        |                                                  | Acidity increase (mgs. KOH/gm.)       | Wt. change (mgs.) | Colour of Specimen                                 |
|          |                                                                                                                                                                                                                                                                                                                                                                        |                                                                                                |                                                      | Specimen                          | Catalyst                                         |                                       |                   |                                                    |
| 18       | Di(3:5:5 trimethyl hexyl) sebacate.                                                                                                                                                                                                                                                                                                                                    | None.....                                                                                      | -252.5                                               | Corroded.....                     | Light peacock.....                               | 10.0                                  | +1.2              | Peacock.....                                       |
| 19       | do.....                                                                                                                                                                                                                                                                                                                                                                | 0.5% Di(3-methyl-4-hydroxy phenyl) thioether.                                                  | +0.6                                                 | Light yellow.....                 | Light brown.....                                 | 0.40                                  | +3.1              | Brown.....                                         |
| 20       | do.....                                                                                                                                                                                                                                                                                                                                                                | { 0.5% Di(3-methyl-4-hydroxy phenyl) thioether.....<br>0.1% Benzimidazole.....                 | +0.8                                                 | Almost clean.....                 | Light peacock.....                               | Nil                                   | -0.8              | Peacock.....                                       |
| 21       | { 47% Di(2-ethyl hexyl) sebacate.....<br>47% Di(3:5:5 trimethyl hexyl) sebacate.....<br>6% Polynonyl methacrylate.....<br>47% Di(2-ethyl hexyl) sebacate.....<br>47% Di(3:5:5 trimethyl hexyl) sebacate.....<br>6% Polynonyl methacrylate.....<br>47% Di(2-ethyl hexyl) sebacate.....<br>47% Di(3:5:5 trimethyl hexyl) sebacate.....<br>6% Polynonyl methacrylate..... | 0.05% Calcium petroleum sulphonate.                                                            | -180                                                 | Light grey.....                   | Bright.....                                      | 15.8                                  | -1.4              | do.....                                            |
| 22       | do.....                                                                                                                                                                                                                                                                                                                                                                | { 0.5% Phenothiazine (technical).<br>0.2% Benzotriazole.....                                   | +0.2                                                 | Trace of light peacock stain..... | Dark peacock with black patches.                 | Nil                                   | +0.2              | Dark peacock/brown.                                |
| 23       | do.....                                                                                                                                                                                                                                                                                                                                                                | { 0.5% Phenothiazine (technical).<br>0.2% Benzotriazole.....                                   | -1.6                                                 | do.....                           | Peacock.....                                     | 0.22                                  | +1.4              | Slight peacock colouration.                        |
| 24       | Di(2-ethyl hexyl) sebacate.                                                                                                                                                                                                                                                                                                                                            | { 5.0% Tri-m-tolyl phosphate.....<br>1.0% Phenothiazine (purified).<br>0.1% Benzotriazole..... | +0.2                                                 | Light peacock.....                | Very dark brown lacquer, almost black in places. | 0.06                                  | +1.6              | 50% Dull black deposit on dark peacock background. |
| 25       | do.....                                                                                                                                                                                                                                                                                                                                                                | { 5.0% Tri-m-tolyl phosphate.....<br>1.0% Phenothiazine (purified).<br>0.1% Benzotriazole..... | Nil                                                  | do.....                           | Light golden.....                                | Nil                                   | +0.2              | Light gold.....                                    |

Tests Nos. 18 and 21 demonstrate the very high acidities developed by uninhibited diesters and blends based on them, with consequent severe corrosion of the cadmium-plated steel specimens. Tests Nos. 19, 22 and 24 show how acidity rise and attack of cadmium-plated steel can be effectively controlled by the presence of antioxidants of the types described, although this is accompanied by an undesirable attack on the copper specimens and catalysts which is particularly severe with phenothiazine. Tests Nos. 20, 23 and 25 show that, by the inclusion in the blends of the inhibitors of the present invention, this attack of copper can be reduced to negligible proportions.

We claim:

1. A lubricating composition consisting essentially of a substantially neutral saturated organic carboxylic acid ester having a viscosity index of at least 100, a pour point not exceeding -40° F., a boiling temperature not less than 600° F., and a flash point not less than 350° F., the said ester being selected from the group consisting of an ester having the general formula



wherein R is a radical selected from the group consisting of saturated aliphatic and cycloaliphatic hydrocarbon radicals having from 2 to 8 carbon atoms, and R<sub>1</sub> and R<sub>2</sub> are radicals selected from the group consisting of branched-chain alkyl and alkyl-substituted cycloalkyl radicals having at least four carbon atoms, and an ester having the general formula



45 icalis having at least 4 carbon atoms, and R<sub>3</sub> is selected from the group consisting of saturated hydrocarbon radicals and polyglycol radicals having not more than 12 carbon atoms; from 0.05 to 5.0% by weight on the weight of the final composition of a compound selected from the group consisting of di(hydroxy aryl) thioethers and dibenzothiazines having good antioxidant properties at 50 elevated temperatures; and from 0.01 to 2.0% by weight on the weight of the final composition of at least one compound selected from the group consisting of imidazole, benzimidazole, pyrazole, benzotriazole and indazole and methyl derivatives of any of the foregoing 55 wherein said methyl groups are substituents of the carbon atoms of the ring.

2. A lubricating composition as claimed in claim 1 wherein said composition contains from 1-15% by weight on the weight of the final composition of a polymer selected from the group consisting of polymers of esters of acrylic and alkyl-substituted acrylic acids.

3. A lubricating composition as claimed in claim 1 wherein said composition contains about 0.5 to about 10% by weight on the weight of the final composition of an additional compound selected from the group consisting of neutral organic phosphate and phosphite esters.

4. A lubricating composition as claimed in claim 1 wherein the ester has the formula



70 75 wherein R is a radical selected from the group consisting of saturated aliphatic and cycloaliphatic hydrocarbon radicals having from 2 to 8 carbon atoms, and R<sub>1</sub> and

## 11

$R_2$  are radicals selected from the group consisting of branched-chain alkyl and alkyl-substituted cycloalkyl radicals having at least four carbon atoms.

5. A lubricating composition as claimed in claim 1 wherein the ester has the formula



wherein  $R_1$  and  $R_2$  are radicals selected from the group consisting of branched-chain alkyl and alkyl-substituted cycloalkyl radicals having at least four carbon atoms and  $n$  is an integer from 2 to 8.

6. A lubricating composition as claimed in claim 1 wherein the ester has the formula



wherein  $R$  is a radical selected from the group consisting of saturated aliphatic and cycloaliphatic hydrocarbon radicals having from 2 to 8 carbon atoms, and  $R_1$  and  $R_2$  are radicals selected from the group consisting of branched-chain alkyl and alkyl-substituted cycloalkyl radicals having at least four carbon atoms, and  $R_3$  is selected from the group consisting of saturated hydrocarbon radicals and polyglycol radicals having not more than 12 carbon atoms.

7. A lubricating composition as claimed in claim 1 wherein the ester is a compound selected from the group consisting of di(3-methyl butyl) azelate, di(2-ethyl hexyl) azelate, di(2-ethyl hexyl) sebacate, di(3:5:5 trimethylhexyl) sebacate, di(3:5:5 trimethylhexyl) azelate, di(1-methyl-4-ethyl octyl) sebacate and 2-ethyl hexyl 3:5:5 trimethylhexyl sebacate.

8. A lubricating composition consisting essentially of a neutral ester having the formula



wherein  $R$  is a radical selected from the group consisting of saturated aliphatic and cycloaliphatic hydrocarbon radicals having from 2 to 8 carbon atoms, and  $R_1$  and  $R_2$  are radicals selected from the group consisting of branched-chain alkyl and alkyl-substituted cycloalkyl radicals having at least four carbon atoms, from 0.1 to 2.0 percent by weight on the weight of the final composition of a dibenzothiazine having good antioxidant properties at elevated temperatures, and from 0.05 to 0.5 percent by weight on the weight of the final composition of at least one compound selected from the group consisting of imidazole, benzimidazole, pyrazole, benzotriazole and indazole and methyl derivatives of any of the foregoing wherein said methyl groups are substituents of the carbon atoms of the ring.

9. A lubricating composition consisting essentially of a neutral ester having the formula



## 12

wherein  $R$  is a radical selected from the group consisting of saturated aliphatic and cycloaliphatic hydrocarbon radicals having from 2 to 8 carbon atoms, and  $R_1$  and  $R_2$  are radicals selected from the group consisting of branched-chain alkyl and alkyl-substituted cycloalkyl radicals having at least four carbon atoms, from 0.1 to 2.0 percent by weight on the weight of the final composition of a di(hydroxyaryl)thioether, and from 0.05 to 0.5 percent by weight on the weight of the final composition of at least one compound selected from the group consisting of imidazole, benzimidazole, pyrazole, benzotriazole and indazole and methyl derivatives of any of the foregoing wherein said methyl groups are substituents of the carbon atoms of the ring.

10. A lubricating composition consisting essentially of a neutral ester having the formula



wherein  $R$  is a radical selected from the group consisting of saturated aliphatic and cycloaliphatic hydrocarbon radicals having from 2 to 8 carbon atoms, and  $R_1$  and  $R_2$  are radicals selected from the group consisting of branched-chain alkyl and alkyl-substituted cycloalkyl radicals having at least four carbon atoms, from 0.1 to 2.0 percent by weight on the weight of the final composition of phenothiazine, and from 0.05 to 0.5 percent by weight on the weight of the final composition of benzotriazole.

11. A lubricating composition consisting essentially of at least one ester selected from the group consisting of di(2-ethyl hexyl) sebacate and di(3:5:5 trimethylhexyl) sebacate, from 0.1 to 2.0 percent by weight of phenothiazine and from 0.05 to 0.5 percent by weight of benzotriazole.

## References Cited in the file of this patent

## UNITED STATES PATENTS

|           |                |               |
|-----------|----------------|---------------|
| 1,805,953 | Morton         | May 19, 1931  |
| 2,370,552 | Lincoln et al. | Feb. 27, 1945 |
| 2,508,617 | Mastin         | May 23, 1950  |
| 2,618,608 | Schaeffer      | Nov. 18, 1952 |
| 2,642,396 | Roddy          | June 16, 1953 |
| 2,692,191 | Haskell        | Oct. 19, 1954 |
| 2,754,216 | Chenicek       | July 10, 1956 |

## FOREIGN PATENTS

|         |               |               |
|---------|---------------|---------------|
| 711,211 | Great Britain | June 30, 1954 |
|---------|---------------|---------------|

## OTHER REFERENCES

- Lubrication Eng., August 1952, pages 177-179.  
 Ind. and Eng. Chem., April 1947, vol. 39, No. 4, pages 491-497.  
 Ind. and Eng. Chem., December 1950, vol. 42, No. 12, pages 2479-2489.  
 Ind. and Eng. Chem., August 1953, vol. 45, No. 8, pages 1766-1769.